

March 19, 1935.

O. W. FROST

1,995,145

MANUFACTURE OF ARTIFICIAL BOARDS AND LIKE STRUCTURES

Filed March 26, 1932



Witness:  
*Chas. H. Housh*

Inventor,  
Orcutt W. Frost,  
By W. Bartlett Jones, Atty.

## UNITED STATES PATENT OFFICE

1,995,145

MANUFACTURE OF ARTIFICIAL BOARDS  
AND LIKE STRUCTURESOrcutt W. Frost, Cloquet, Minn., assignor to  
Wood Conversion Company, Cloquet, Minn., a  
corporation of Delaware

Application March 26, 1932, Serial No. 601,411

5 Claims. (CL. 92—41)

The present invention relates to fiber products, such as insulation for heat and sound, and to artificial lumber, such as boards, shingles, and like forms which may be cut up, and to formed or molded articles of various sizes and shapes which may or may not be suitable for size reduction.

It has particular reference to the forming of board, or sheet material of uniform thickness, that is with parallel surfaces, which can be cut into various sizes and shapes for use as a substitute for sawn lumber. Such material is hereinafter referred to as "sheet lumber".

Dense hard boards of the prior art which are used as artificial lumber, or wall board, and which are formed of wood fiber, or other cellulosic material, are ordinarily heavier and denser than ordinary sawn lumber. The latter averages about 30 lbs. per cu. ft. while the artificial boards referred to run from 40 to 50 lbs. per cu. ft., some being well known which have a density of 1, or over 60 lbs. per cu. ft. Much of the material is so compressed and located that it is not efficiently used in carrying stresses. By the present invention, the material is so allocated in a structure that less dense, and stronger sheets may be made from the same amount of material.

An important feature of the invention as it is used in connection with sheet lumber, is the use, of a core layer, and of one or two surfacing layers of suitable material. The invention incorporates in artificial fibrous products, the principle of mechanics which is effective in steel structures, such as channel bars, angle bars, T-bars, H-beams, I-beams, and the like, wherein great strength is obtainable with a minimum of material.

In other words, in the present invention, the material is so composed, and/or formed that it is most efficient where strength is required. In particular for "sheet lumber", at least one strong surface layer is backed by a skeleton structure or two such layers have a skeleton connecting core.

Heretofore, artificial boards or sheets have been made of fiber by simultaneously compressing and completely or partially drying a wet homogeneously mixed mass of fibrous cellulosic material. Among the materials heretofore employed are: natural wood fibers, mechanically ground wood, semi-chemical pulp, chemical cellulose, waste paper, commercial fiber waste, such as bagasse, and other forms. In using these materials to make sheets by application of heat and pressure to wet masses of the fibers, the mass itself acts

as a plastic body and dries into a unitary body. Sometimes a binding agent is added, or one may be present in the fiber mass, naturally, or formed therein by the process employed. From experiments which I have conducted I have shown that when the fibers of wood, ligno-cellulose, or cellulose are hydrated by working mechanically in water, the self-cementing action of the fibers increases with the amount of hydration. In this invention I may employ such hydration processes to increase the self-cementing properties of a cellulosic material, or I may add a cementing agent, or the cementing agent may be derived from the fibers during the process.

The sheets made heretofore have employed a substantially uniform mixture of base materials. The sheets, or other shapes, have been made in varying thicknesses, and of varying degrees of hardness, or density, largely by varying the amount and duration of heat and pressure. Boards have been made, for example, by applying heat and a following-up pressure until the sheet is thoroughly dry. The pressure applied in part effects the density. A substantially uniformity may be obtained throughout the thickness of the sheet. Other sheets have been made with cessation of heat and pressure, either one or the other, or both, before complete drying of the sheet, so that the outside surfaces have a different texture than the interior.

One defect of such prior articles is the utilization of the same materials on the entire interior of the board or sheet as is used on the exterior. The requirements and the functions of the outer layers and the inner layers are not the same, and the differences are such that the inner layer in particular may be in part dispensed with, and may include cheaper material.

Another defect of prior art materials is the necessary density for the required strength. Where thick boards are desired, too much material is wastefully used in the prior art processes and structures.

One object of the present invention is the provision of a board or like article having at the surface material suitable for the requirements of the surface, and a less dense and a cheaper body supported and carried by the material of the surface, said surface material extending into the body and connecting the two surfaces.

Another object of the invention is the provision of a skeleton core in a board or like article.

One particular object of the invention is the provision of voids in the core of the article.

Another particular object of the invention is the

provision of coarser elements in the core than in the surface.

Still another particular object of the invention is the provision of a core of shreds of material, such as wood, for example "excelsior", as a filling material of the supporting core.

Another object of the invention is the making of a composite structure by separately making (1) a core-forming base, and (2) one or two surface-forming bases, combining them after they have assumed some independent form, and thereafter treating the composite structure to produce a unitary, composite structure.

The present invention may be carried out in numerous ways, and differently appearing structures may result, all of which, however, involve the fundamental idea of this invention.

Thick boards, like lumber, are frequently desirable, but the prior art processes of making thick boards are not economically adapted for operation to effect this result. Thick boards are frequently desirable, because the transverse strength is proportional to the square of the thickness, and the surfaces bear the greatest stresses. Just as an I-beam becomes stronger by increasing the width of the web connecting the flanges, so the board of the present invention becomes stronger by increasing the thickness of the skeleton core between the surface layers. In making boards or "sheet lumber", or like articles, by the present invention, I provide at least one sufficiently strong surface layer, but preferably two, and a backing or connecting core of sufficient strength to support or carry the surface layer or layers, or the "stress" layer, as it will hereinafter be referred to. In sheet lumber, two parallel stress layers are carried and connected by a suitable core. The greatest variations in the invention as herein described are variations in the character and formation of the core. Of course, a stress layer may vary widely in density, composition, and other properties, just as the artificial sheets of the prior art may vary.

In connection with the general and detailed description of methods, apparatus and products, which have been chosen to illustrate the present invention, the accompanying drawing is referred to. In the drawing:

Fig. 1 illustrates diagrammatically the arrangements of mechanical elements which may be used in carrying out the invention.

Fig. 2 represents an artificial board containing in the core particles like sawdust as a filler.

Fig. 3 represents a similar product containing in the core shredded particles, such as excelsior.

Fig. 4 represents an artificial board in which the filler comprises systematically arranged solid elements such as wooden strips.

Fig. 5 represents an artificial board in which voids are formed by removal of the elements present in the core during formation of the board.

Fig. 6 represents an artificial board in which there is an intermediate layer like a surface layer sandwiched between two core layers.

The materials for the stress layer may be the same as is used in any prior art board, and may include fiber and a cementing agent. The latter may be added, or may be by nature an ingredient accompanying the original fiber source, or may be one formed incidentally or intentionally in the process of preparing the fiber. I prefer to use a cellulosic fiber, and to treat it by a hydrating process to form a cellulose hydrate. This may be a gelatinous film on some or all of the fibers, or it may be a liquid mass of completely gelatinized

fibers added to less hydrated, or to unhydrated fibers. I prefer to use as the body of the fiber, a partially digested wood, or semi-chemical pulp, such as ligno-cellulose, so termed to distinguish it from more completely cooked wood which is substantially "cellulose" in character. Where wood, or wood waste, or straw and the like as a raw material, is cooked with chemicals, ligno-cellulose is preferred to cellulose, because of the higher yield of fiber to be obtained. Where hydration is practiced to form pulp-bonding material, either ligno-cellulose or cellulose may be hydrated. If ground wood pulp, or other mechanically undigested wood, or other cellulosic material, is employed, hydration of the cellulosic material may be effected, irrespective of the specific character of the cellulosic material.

As material for the core, any kind of pulp may be used. The core may contain the same kind of pulp as the stress layer and such material in the core and stress layer may be continuous. The pulp part of the core has the same or substantially the same density as the pulp in the stress layers, but the core as a body may have an average density which is less than the density of the stress layers. The non-pulp part of the core may be void space, or any filling material either granular or fibrous, and preferably, if fibrous, it is to be in the form of aggregates of fibers rather than fibrated material. Flakes of paper, coarse sawdust, shreds of wood, wood shavings, slivers of wood, and the like, may be used. Excelsior is most desirable because of its flexibility. A very coarse grade of such excelsior may be used. It is to be understood that a pulp cementing agent is present in the pulp part of the core to bind the pulp part together into a network, or a unit around a filler. Preferably, such cementing agent is the same as is used in the pulp of stress layer, and a hydrated cellulose is suitable for both. By using the same bond in the pulp of the stress layer and in the pulp of the core an integral substance is established extending as a skeleton or net work throughout the unit, and it may be made integral by the one process of uniting and curing the different elements of the composite structure.

In practicing the invention the weaker core may be effected by creating voids therein, either systematically, as by some mechanical means, or heterogeneously, as by controlling the character of its composition. In the mechanical method I may incorporate solid material as a part of the structure to define the voids and to resist and to transmit compression, and then remove the solid means, either bodily, in fragments, or otherwise. I may use elongated rods or bars which may be removed endwise from the voids formed thereby in the completed product. I may use volatile or decomposable crystalline material, which remains in solid form in the process, and remove it wholly or partly as a gas or vapor through the pores of the completed unit. I may use a leavening agent in the core which may be either soluble or insoluble in water.

While any solid may be used, such as sand, mineral fibers, animal fibers, and metal shreds or fibers, I prefer waste products, and especially light-weight waste, such as material which is less dense than pulp parts in their ultimate form. Coarse sawdust, shavings, or shredded wood, exemplified by coarse excelsior, are suitable light-weight materials. The more elongated is the form of such filler, the more it functions as a mechanical reinforcement. It is of such a char-

acter that when compressed it forms interstices, which in the final product are filled with cemented pulp integrally united to cemented pulp in the stress layers.

5 To make such a board, I form a pulpy mass, preferably by treating wood waste, in any way to form a wet fibrated mass. The fibration may be mechanical, chemical, or both. Ground wood may be used. Cellulose pulp, such as paper stock, may be used. 10 Semi-chemical pulp may be used, such as wood chips softened by a partial chemical digestion, and then mechanically separated as in a rod mill. All or part of the pulp may be treated to form cellulose hydrate, as by the mechanical 15 action of a beater (Hollander), a Clafin, or a Jordan, or otherwise. A part of the pulp, or any other cellulose pulp, may be completely hydrated to a gelatinous solution without fibrous form, or it may be very highly hydrated, and such cellulose hydrate may be added to less hydrated pulp or to unhydrated pulp. By any method, a self-cementing pulp mixture is formed, exemplified by a mixture of fibre, or pulp, and gelatinous cellulose hydrate. Preferably all the fibers are hydrated to form a gelatinous skin about each of them. Such material is a plastic mass when wet, flowing as a plastic mass.

The plastic mass described is used in part by itself to form wet pulp laps for the surface layers. 30 It is also used as the essential part of the core in admixture with the solid filler. For example 60% of shredded wood and 40% of self-cementing pulp (air dry weights) form a suitable core. In practice three machines are used, one to form the wet mat of core, which may be about 2 inches thick, and two others, such as cylinder machines, one above and one below the core former, for forming and discharging a wet lap of adhesive pulp onto the opposite surfaces of the wet core 35 lap. The surfacing laps may be  $\frac{1}{8}$  inches thick when wet. The three laps are united, pressed through squeeze rolls to eliminate surplus water, and then passed to a press. The process may be continuous, or intermittent according to machines employed. If intermittent the formed 40 sheets may be made initially of size suitable for the press. If continuous, the composite sheet may be cut to fit the press.

Multiple presses suitable for the process are 45 well-known and some may operate simultaneously upon as many as twenty such sheets. They are capable of using pressures up to 1500 lbs. per sq. inch, and of being heated by steam at a pressure up to 100 to 150 lbs. per sq. inch. They may also be electrically heated.

The pressure and temperature which may be employed generally are not critical in practicing this invention and may be varied according to the results desired. For certain products fixed 50 conditions may be specified. It is preferred that the temperature should be sufficient to boil out the excess water. Air drying or evaporation is not excluded, however, and it may be desirable for certain special types. It has been found that the 55 air-dried product is better when hydrated cellulose is present, as the concentration of the hydrated or gelatinized cellulose is increased. The pressure should be sufficient to secure the desired density. Pressures from 50 to 1200 lbs. have been 60 used with a corresponding variety of resulting products. A steam pressure of 100 pounds per sq. inch and a mechanical pressure of 250 lbs. is satisfactory for a general purpose sheet lumber. When pressure and a boiling temperature are applied, the applications are preferably simultane- 65

ous, and are continued until liquid water in the mass has been boiled out. Such drying converts the cellulose hydrate into a hard horny mass which is integral as a continuous mass or network from face, through core to face, being substantially uniform in character through its integral extent.

The following table shows the properties of a board made by this process, generally as described above, using a mechanical pressure of 75 10 lbs. and a steam gauge pressure of 100 lbs. in the platens as compared to a reference board (item I) made by the prior art processes, of uniform density from face to face, with the same pulp mass.

| Item   | Pounds bonded pulp per sq. ft. | Composition                                                  | Thickness face to face | Pounds per cu. ft. | Breaking point under transverse load applied at center of 6 in. span 4 inches wide |
|--------|--------------------------------|--------------------------------------------------------------|------------------------|--------------------|------------------------------------------------------------------------------------|
| 1..... | .635                           | Per cent<br>100 pulp...<br>55 pulp...<br>45 shred...<br>wood | .137 in.               | 43.5               | 46.7 lbs.                                                                          |
| 2..... | .432                           | 45 pulp...<br>55 shred...<br>wood                            | .260 in.               | 31.0               | 85.5 lbs.                                                                          |
| 3..... | .573                           | 45 pulp...<br>55 shred...<br>wood                            | .553 in.               | 25.6               | 136.0 lbs.                                                                         |

The foregoing table clearly demonstrates that a less dense board containing a less quantity of bonded pulp, may be stronger than the same area of board containing more of such pulp.

As a detailed example of carrying out the invention in the manner generally described above, the following description will suffice.

Ordinary paper pulp, such as low stock or other pulp used in the manufacture of insulating boards is mixed with a suitable filler in a desired proportion, such as 40% pulp and 60% sawdust. The actual ratio may be determined by the desired characteristics of the resulting product. The mixed mass in wet plastic form 40 is felted in a suitable machine, such as a cylinder machine, like the Oliver, designated 10 in Fig. 1. A continuous felted sheet 11 is thus discharged and may be couched over to a conveyer belt, preferably in the form of a screen 12, 50 under which there is a suction box 13. The mat is thus made more dense and less wet.

Additional felting means, such as Olivers 15 above the mat 11 and 16 below the mat 11, form thinner sheets or mats 17 and 18 of pulp, preferably identical with that used in admixture with the sawdust. These laps are couched to conveyer belts 19 and 20 to bring them toward the core-mat 11, at which they are properly directed to form facings on the core mat. The three mats move uniformly together as one sheet 21 over a conveyer 22, preferably a screen, to squeeze rolls 23 for removal of surplus water, and for a uniting compression of the mats. The sheet may then be cut into sizes suitable for the 60 hot press. In the press they may be subjected to a continuous pressure of 250 pounds per square inch, and a drying heat produced by a 70 pound steam pressure within the platens of the press.

Fig. 2 represents the product in cross-section. The product has three zones 25, 26 and 27, of which 26 is the core. The surface zones 25 and 27 are substantially pulp layers, and the pulp substance extends from one layer to the other, 75

through the core as an integral substance, designated in the core as 28. The parts 29 designate the sawdust, and represent generally whatever filler may be used. One surface layer in the press may be formed against a wire screen on the platen, as is well known, for aiding the liberation of steam in the drying process. Screen markings 30 are designated.

In the manufacture above described it is not necessary to form two stress layers. The lower Oliver 16 and its product 18 may be omitted, and to some extent a less definite stress layer having a uniform surface, will be formed by gravity drainage of the pulp substance to the lower side of the unit. The ultimate essential characteristics will however prevail in the resulting product.

Where a water-proofed product is desired the surface layers 17 and 18 may be suitably treated or sized, either in the pulp form before felting, or after felting, as desired. When such treatment is limited to the pulp in the stress layers only, there is economy in sizing materials as compared to sizing all the pulp for the board, as practiced heretofore for the uniform type of boards.

In Fig. 3 a similar product is shown in which shreds of wood such as "excelsior" 32 is present in the core, contained in the hardened integral matrix 33 which is comprised in the surface layers and which fills the interstices between the shreds.

Fig. 4 represents a departure from the forms of Figs. 2 and 3, in which the filler is systematically arranged. Wooden strips 35 of triangular cross-section are arranged in complementary relation as shown. These may be left embedded in the product. The pulp 36 extends integrally from face layer 37 to face layer 38, and between the adjacent lengths of filler in the form of webs 39. In manufacture various expedients may be adopted for incorporating the filler. It is to be noted that prior to compression in the press, the adjacent lengths may be more separated along the line of the thickness of the board, and in the process of compression the faces 40 and 41 aid in compressing the pulp in the web.

In Fig. 5 a further modification is shown, similar in original form to that of Fig. 4. Rods such as round metal rods 42 may be inserted in the core base and housed therein as the filler. They may thereafter be withdrawn, leaving voids indicated as 43 in the core, to reduce its average density. Thus the entire substance 44 of the core and the stress layer is the same, is integral, and of the same density, but because of the voids, the average density of the core is less. Likewise, strips shaped as in Fig. 4 may be withdrawn, and they may be originally supplied as metal rods, as in Fig. 5 for the purpose of easy withdrawal. The contraction of metal on cooling contributes to the separation of the rods from the pulp in the core.

In Fig. 6 it is shown that the invention is not limited to unfilled layers at the surface. Such layers may be arranged within the core in one or more layers, exemplified by a single layer of pulp 46 sandwiched between two core layers 47 and 48, the whole being integrally united by the pulp substance with two surface layers 49 and 50 of pulp base.

In general discussion it may be stated that the sawdust particles, and the shredded wood of Figs. 2 and 3, respectively, are not necessarily cemented to the pulp substance, and may be

found quite free therein, as if each resides in a void. They function in the process of forming as pressure-distributing means and as means for forming "voids" in the integral substance. Because of the cheap character of the filler, it may be left in the voids which it creates, and it is not detrimental to the desired character of the product if the filler particle draws away from and resides more or less loosely or detached in the void. The forms of Figs. 2 and 3 are the preferred forms for reasons of simplicity and economy in the process of manufacture.

The product may exhibit a characteristic laminated structure in the plane of the sheet at any part of the body, but this is to be distinguished from the existence of separable and distinct layers. Because the compression is unilateral and not cubical such laminations may readily occur to the extent that the fibers, or the filler, are elongated in character.

In general discussion of the process of formation, it may be stated that mechanical pressure is not essential in drying the cellulose hydrate to a hard horny cementing mass. It is material to the density of the product and the intimate relation of the compressed fibers to each other and to the horny cement. Likewise, high temperature is not essential to the formation of the hard and horny mass from hydrated cellulose. It is material to the speed of drying. The transfer of heat to the interior is quicker by higher heat. In the case of metal inserts the transfer of heat to the interior is quicker than in the case of less conductive filler in the core, such as wood, sawdust, shavings, shredded wood. The latter absorb some water, and this also must be driven off as well as the water in the self-cementing pulp.

The invention is not limited to any particular thickness of the stress layers, or the core, or any particular ratio of thicknesses. A very thin face layer may be used, and some decorative features may result in regulating thicknesses. For example, when the stress layers are sufficiently thin, the pressure means in the core, whether rods, grids, sawdust, shredded wood, or whatever may be used, can be made to exhibit shadowy or clear-cut markings in the exposed face, due to slight deviations from equal distribution of pressure. Particularly with shredded wood a variegated net work of lines may appear having slightly darker shade where lengths of shredded wood press against the surface layer. Colors may be incorporated into the surface layer, and may also, if desired, be incorporated into the shredded wood to be preferentially squeezed therefrom into the surface layers to cause a mottled design in color.

The chips or other filler may be previously coated with a water-excluding substance, or otherwise treated to prevent useless absorption of water from the aqueous pulp. Paraffin may be used, and will so function until heat is applied. Upon application of heat the paraffin will melt and it is then distributed throughout the board by diffusion, making the final product more water-resistant. I have found that paraffin and any similarly acting material increases the drying time because of the subsequent diffusion under heat. However, when a suitably heat-resistant substance like gilsonite is used to render the filler water-resistant, the time of drying may be shortened, because there is no water in the filler to be removed.

The product may be made with the particular

object of providing high thermal insulation properties. The less dense is the board, the more air space there is within it, and hence the more effective it is as a heat insulation. 5 The forms which have large voids therein, such as unfilled air spaces, and the more spongy forms, are particularly advantageous as heat insulation. It is also to be understood that the sound transmitting property is lessened, and the 10 sound absorbing quality is increased, by the same factors which increase the heat insulating capacity. In other words, the acoustical and the thermal properties may be advantageously increased by decreasing the average density of 15 the product.

Products of the present invention may be made to approximate lumber in physical characteristics, and may or may not be grained to some degree, according to the character of the 20 filler. It has greater strength per unit weight than the boards of uniformly dense material. Because of the use of filler as described, the product may be made in thicker form with less 25 problems incidental to drying than are met with in making boards of the same thickness from uniformly homogeneous pulp masses. The boards are cheaper to make per unit of thickness. There is less warping, expansion and 30 contraction because of the lower average density of the core. The board will receive and will hold 35 nails at the edges, without splitting. The product has a higher thermal insulating value than the denser forms. It may have an attractive 40 surface appearance subject to variation by slight changes in proportions and in materials 45 employed in the process of construction. When sizing is desired, economies may be effected.

It is also to be understood that sizing and 45 water-proofing agents may be incorporated into 50 any of the laps for the surface, or the core. Materials for such purpose are well known. The fibers employed may be proofed against water, fire, insects, and rot in any known manner, if desired, and such other changes and modifications, and prior art practices may be adopted, without departing from the invention as expressed in the appended claims.

I claim:

1. The method of making an artificial board-like product which comprises making a wet core by forming around particles of a filler a skeleton 55 network of wet fibrous composition capable of a self-cementing action on drying, forming on said

core a wet surfacing layer consisting substantially entirely of fibrous composition having cementing properties similar to the fibrous composition of the core, pressing the core and surface layer together, drying the resulting body into an integral unit, and removing the filler to leave voids 5 in said core portion of the unit.

2. The method of making an artificial board-like product which comprises making a wet core by forming around elongated rod-like elements 10 a wet fibrous composition capable of a self-cementing action on drying, forming on said core a wet surfacing layer consisting substantially entirely of fibrous composition having cementing properties similar to the fibrous composition of 15 the core, pressing the core and surface layer together, drying the resulting body into an integral unit, and removing the rod-like elements from the core.

3. The method of making an artificial board-like product which comprises making a core by forming around filler elements a skeleton network of a self-cementing mass of structural composition, forming on said core a surfacing layer consisting substantially entirely of the essential composition of said core, treating the united core and layer to cause setting and integral union of 20 said core and layer by its self-cementing action, 25 and removing the filler elements.

4. The method of making an artificial board-like product which comprises making a core by forming around filler elements a skeleton network of fiber and cementing bond, forming on said core a surfacing layer consisting substantially entirely of fiber and a cementing bond having cementing 30 properties similar to the cementing bond of the core, treating the united core and layer to effect 35 setting of the cementing bond and integral union of the core and layer, and removing the filler elements.

5. The method of making an artificial board-like product which comprises making a core by forming around filler elements a mass of highly hydrated cellulose and fibers, forming on said core a surfacing layer consisting substantially entirely 45 of highly hydrated cellulose and fibers, treating the united layer and core to heat and pressure to dry and to compress the drying mass, whereby to form a hard integral substance at the surface extending as a skeleton through the core, and 50 removing the filler elements from the core.

ORCUTT W. FROST.